

Dec. 1, 1942.

E. FLEISCHMANN

2,303,449

JACKETED BULLET

Filed Nov. 21, 1939

*Fig.1.*



*Fig.2.*



*Fig.3.*



*Fig.4.*



INVENTOR

Ernst Fleischmann  
by his attorneys  
Stebbins and Blenko

## UNITED STATES PATENT OFFICE

2,303,449

## JACKETED BULLET

Ernst Fleischmann, Clairton, Pa., assignor to  
Copperweld Steel Company, Glassport, Pa., a  
corporation of Pennsylvania

Application November 21, 1939, Serial No. 305,495

3 Claims. (Cl. 102—47)

This invention relates generally to projectiles and particularly to a jacketed bullet such as a fle bullet or the like.

It has been recognized heretofore that the provision of a jacket of relatively soft material on a bullet of relatively hard material such as steel or the like, reduces ricochetting and increases penetrating power. Copper-jacketed steel bullets, for example, have been used and show a deeper penetration than a steel-jacketed lead bullet. Difficulty has been experienced, however, in maintaining the copper jacket precisely concentric with the body portion of the bullet, when rolling a copper clad billet down to rod stock suitable for the manufacture of bullets. Because of the difference between the specific gravities of copper and steel, any lack of concentricity of the jacket with respect to the body renders the bullet slightly unbalanced, i. e., the center of gravity of any transverse section does not necessarily coincide with the geometrical center of the section. Such unbalance causes the bullet to deviate from a straight line when firing and thus reduces the accuracy of fire considerably.

I have invented a novel jacketed bullet which overcomes the aforementioned objection. In a referred embodiment the bullet of my invention comprises a core or body portion of suitable material, e. g., steel, and a jacket of relatively softer material. The jacket is composed of metal having a specific gravity substantially the same as that of the material of which the body portion or core of the bullet is composed. Thus any lack of concentricity between the body or core and the jacket will not render the bullet unbalanced. The center of gravity of any transverse section will coincide precisely with the geometric center thereof.

The accompanying drawing illustrates a preferred embodiment of the invention. In the drawing,

Fig. 1 is a side elevation of a jacketed bullet according to the invention;

Fig. 2 is a transverse section thereof taken along the plane of line II—II of Fig. 1;

Fig. 3 is a longitudinal section therethrough taken along the plane of line III—III of Fig. 1; and

Fig. 4 is a view similar to Fig. 3 showing a modification.

Referring in detail to the drawing, a jacketed bullet indicated generally at 10 comprises a body core 11 and a sheath or jacket 12. As shown in the drawing, the sheath is not concentric with the core or, stated differently, the thickness of

the sheath is not uniform at all points around the circumference of the bullet. This is a condition frequently encountered in manufacturing composite bar stock such as that from which the bullet 10 may best be made. The sheath is bonded to the core by any suitable method so that the bullet as a whole is a unitary object. The core 11 is preferably of steel.

The metal of which the jacket 12 is composed may be of any suitable composition so long as it has a specific gravity substantially the same as that of steel, i. e., approximately 7.88. One metal which is suitable for the purpose is an alloy of copper, aluminum and iron comprising about 90% copper, 8.5% aluminum, and 1.5% iron. This alloy has a specific gravity of 7.79 which is sufficiently close to that of steel to preclude any unbalance resulting from slight non-uniformities in the thickness of the jacket at various points around the body or core.

If the body of the bullet is composed of metal other than steel, the metal of which the jacket is composed will be chosen so that its specific gravity conforms as closely as may be to that of the metal of which the body is composed.

Bullets made in accordance with the invention may be of any desired shape or size for various applications and may be manufactured by the same methods and apparatus as used heretofore for making jacketed bullets.

The bullets may, for example, be turned down from bar stock as shown in Figure 3 or swedged down, either hot or cold, as shown at 10' in Figure 4. In the former case, the jacket is removed adjacent the nose of the bullet by the turning operation. In the latter case, the jacket is merely thinned slightly adjacent the nose.

Bullets made in accordance with the invention are characterized by the desirable qualities of bullets known heretofore having a jacket of a metal relatively softer than the body, such as reduction in ricochetting and increased penetrating power. They also have the further advantage above pointed out, viz., the higher firing accuracy made possible by elimination of the unbalance resulting from slight non-uniformity in the thickness of the jacket or lack of concentricity between the jacket and body. The invention thus makes it unnecessary to guarantee an absolutely uniform thickness of coating, in order to preclude the unbalanced condition thereby facilitating the manufacture of bullets and reducing the cost thereof.

Although I have disclosed herein but a preferred embodiment of the invention, it will be

understood that slight departures from the general principle thereof may be made within the scope of the appended claims.

I claim:

1. A jacketed bullet comprising a steel body and a jacket composed of an alloy comprising about 90% copper, 8.5% aluminum and 1.5% iron.
2. A bullet having a core or body of steel and a jacket thereon composed of an alloy which

is predominantly of copper and has substantially the same density as steel.

3. A bullet having a metal core or body and jacket thereon composed of an alloy predominantly of copper and having substantially the same density as the metal of which the core or body is composed.

ERNST FLEISCHMANN.